

G. W. WALLACE.

PROCESS FOR DISTILLING CARBONACEOUS MATERIAL.

APPLICATION FILED JUNE 16, 1919.

1,358,664.

Patented Nov. 9, 1920.



FIG. 2



FIG. 3



GEORGE W. WALLACE,

by Bakewell, Church Atty's.

# UNITED STATES PATENT OFFICE.

GEORGE W. WALLACE, OF EAST ST. LOUIS, ILLINOIS.

## PROCESS FOR DISTILLING CARBONACEOUS MATERIAL.

1,358,664.

Specification of Letters Patent.

Patented Nov. 9, 1920.

Application filed June 16, 1919. Serial No. 304,417.

To all whom it may concern:

Be it known that I, GEORGE W. WALLACE, a citizen of the United States, residing at East St. Louis, Illinois, have invented a certain new and useful Improvement in Processes for Distilling Carbonaceous Materials, of which the following is a full, clear, and exact description, such as will enable others skilled in the art to which it appertains to make and use the same.

10 This invention relates to the carbonization or distillation of solid carbonaceous materials, such, for example, as coal, lignites and other fusible bituminous substances.

15 When coal is carbonized or distilled in a closed chamber or retort provided with a take-off duct arranged at the coolest portion of the charge and constituting the sole outlet for the gases, vapors and liquids evolved 20 in the distilling operation, the coal in the retort becomes coked progressively, as the heat penetrates inwardly through same, the heat causing the coal to fuse into a molten mass and then solidify gradually into permanent 25 coke. As the distilling operation proceeds, the coking zone, represented by the fused or molten mass, moves inwardly progressively toward the take-off duct or collection chamber at the coolest portion of the charge, thus

30 leaving a body of coke in the zone lying outside of the coking zone. At the beginning of the operation the coal in proximity to the wall of the retort, to which the heat is applied, first softens and starts to give off

35 gases high in methane and oils that are light in gravity and very volatile, most of the moisture in the coal being driven off at this period of the operation. As the temperature is elevated the coal begins to melt and

40 turn into a putty-like mass, and when a temperature of approximately 650° F. to 750° F. is reached, the coal is a boiling, bubbling mass. Thereafter, this boiling, bubbling mass gradually solidifies or

45 changes into permanent coke. At the completion of the coking stage or at the first stage of the conversion into permanent coke, the mass is dense, impervious and in the form of a relatively thin layer or wall of

50 solidifying material that extends vertically through the retort, and which acts as a barrier between the boiling, bubbling mass in the coking zone and the permanent coke or material lying on the other side of said barrier which has passed through the coking

stage. In numerous tests that I have made with various kinds of coal, I have found that the vertical barrier just referred to is usually less than one-eighth of an inch in thickness and that it conforms approximately to the shape of the heated wall of the retort and extends vertically throughout the entire height of the body of material in the retort. Hence, said barrier effectively cuts off the escape into the take-off duct of any gases that continue to evolve from the material outside of the coking zone which has passed through the coking stage. I have also discovered that any disturbance of the thin barrier or layer of solidifying coke adjacent the molten mass in the coking zone, such, for example, as the passage through said barrier of gases that are evolved on either side of the barrier, has a permanent effect on the structure of the coke and produces coke that is fragile and in the form of small pieces. This is due to the fact that the passage of gases through said solidifying mass forms cracks in same which develop into wide fissures when the material constituting the barrier sets or shrinks during the last stage of the conversion into permanent coke.

55 If the volatile matter that is continually escaping from the boiling, bubbling mass in the coking zone, consisting of most of the oily hydrocarbons and probably 50% of the gases that are evolved from the coal, is allowed to follow the path of least resistance in escaping from the distilling chamber, 60 there is a tendency for said gases to break through the barrier adjacent the bubbling mass of coal and flow outwardly through same, instead of in the opposite direction through the material lying between the take-off duct and the boiling, bubbling mass in the coking zone, due to the fact that said material is more impervious than said barrier and is composed of partially melted coal of putty-like consistency and green coal that 65 is impregnated with pitchy oils and condensed viscid products that have become mixed with the green coal. The passage of any gases outwardly through said barrier not only forms fissures in the barrier, thus 70 producing a poor quality of coke, as previously described, but the passage of gases outwardly through said barrier also causes the volatile matter evolved from the coal to come in contact with the incandescent coke 75

60

65

70

75

80

85

90

95

100

105

110

115

lying outside of the coking zone, and thus undergo secondary decomposition, thereby destroying much of the oil and gas and forming free carbon and lamp black along with gaseous hydrogen, which is the poorest of all artificial gases from a heat unit standpoint.

The passage of the gases and vapors outwardly through the barrier adjacent the boiling, bubbling mass in the coking zone can be prevented by creating a suction in the take-off duct of sufficient intensity to overcome the resistance offered by the putty-like mass of partially melted coal and the mass of pitch impregnated coal lying between the take-off duct and the coking zone, but even when a suction is employed to draw the gases, vapors and liquids into the take-off duct, there is still considerable danger of the thin barrier of solidifying material in the coking zone being disrupted, due to the passage inwardly through said barrier of gases that continue to evolve from the material lying outside of the coking zone. Furthermore, there is a tendency for the gases that continue to evolve from the material that has passed through the coking stage to build up pressure in the retort and crack the retort, if it be made of clay or silica, thus permitting fuel gases to come in contact with the gases and liquids evolved from the coal and ruin said evolved gases and liquids.

Accordingly, in distilling coal in a closed retort or distilling chamber provided with a take-off duct or collection chamber that constitutes the sole outlet for the evolved gases, liquids and vapors, it is essential to prevent the solidifying material in the coking zone from being disrupted by the passage through same of gases that are evolved either from the material in the coking zone, or from the material that has passed through the coking stage. Furthermore, when a suction or partial vacuum is used in the take-off duct to withdraw the gases, vapors and liquids evolved from the material in the coking zone, it is necessary to prevent said suction from being exerted on the outside of the barrier adjacent the molten mass in the coking zone, namely, the side nearest to the heated wall of the retort, as any suction exerted on the outer side of said barrier tends to cause the gases evolving in the coking zone to force their way outwardly through said barrier, due to the greater resistance that the material lying between the take-off duct and the molten mass offers to the passage of such gases.

My invention has for its main object to provide a practicable process for distilling or carbonizing fusible bituminous substances that insures the production of a good grade of coke, even from inferior qualities of cok-

ing coals, and which also insures the recovery of a high percentage of the oils and volatile constituents in bituminous substances.

Another object is to provide a rapid process for distilling or carbonizing fusible bituminous substances that can be accurately controlled and which can be practised in a retort or distilling chamber formed of refractory material such as clay or silica.

To this end I have devised a process for distilling, carbonizing or vaporizing solid carbonaceous material which is characterized by subjecting a continuous body of material of the character mentioned to such treatment in a retort or closed distilling chamber that the gases, vapors and liquids which are evolved from the material passing through the coking stage will travel through the coolest portion of the material in the distilling chamber in escaping therefrom and providing unobstructed passageways in the material in the distilling chamber through which gases can escape from the zone lying outside of the coking zone without disrupting the solidifying material that is changing into permanent coke. The gases and liquids that are evolved from the material passing through the coking stage are preferably drawn into a take-off duct or collection chamber located at the coolest portion of the charge by means of a slight suction or vacuum which also assists in collapsing the bubbles in the molten mass in the coking zone, as said molten mass gradually changes into a solid state, and the passageways that are provided for the escape of the gases which continue to evolve from the material that has passed through the coking stage are so formed that there is no liability of their becoming obstructed and no liability of the suction being exerted on the outer side of the thin barrier of solidifying material adjacent the molten mass in the coking zone, in a direction tending to cause the gases and vapors evolving from said molten mass to pass outwardly through said barrier.

My present process is similar to the process described in my prior U. S. Patent No. 1,283,001, dated October 29, 1918, in that it provides for distilling solid carbonaceous material in a closed distilling chamber in such a manner that the evolved gases, vapors and liquids travel through the coolest portion of the material in said chamber into a take-off duct, and thence immediately escape through said take-off duct before secondary decomposition can occur, preferably downwardly to an eduction pipe communicating with the lower end of said take-off duct, but it differs from my said prior process in that it contemplates providing means for keeping the solidifying material in the coking zone intact and permitting the

escape into the take-off duct of any gases that continue to evolve from the material which has passed through the coking stage.

The apparatus that I have herein illustrated for practising my present process forms the subject-matter of my divisional application Serial No. 390,187, filed June 19, 1920, and consists of a closed distilling chamber or retort, a take-off duct or collection chamber arranged preferably inside of said distilling chamber at the center of same and of the same general contour as the side wall of the distilling chamber, the lower end of said take-off duct communicating 10 with a suction-producing device, and members projecting radially from said take-off duct into the material in the distilling chamber and constructed so that they form unobstructed passageways extending through 15 the coking zone, through which gases can travel into the take-off duct from the zone outside of the coking zone. Various other forms of apparatus can be used, however, for practising my process, and therefore I 20 do not wish it to be understood that my process is limited to use with an apparatus of the particular construction herein shown. Figure 1 of the drawings is a vertical sectional view of one form of apparatus that 25 can be used in practising my present process.

Fig. 2 is an enlarged detail sectional view, illustrating the construction of one of the radially-projecting devices on the take-off 30 duct that forms a passageway extending outwardly from the take-off duct through the coking zone; and

Fig. 3 is a cross-sectional view, taken on the line 3—3 of Fig. 2.

The apparatus shown in Fig. 1 comprises 35 a closed distilling chamber or retort A that is adapted to contain a continuous body of solid carbonaceous material, means for externally heating said chamber, such, for example, as a combustion chamber B to which products of combustion are supplied and arranged in proximity to the side wall of the chamber A, a take-off duct or collection chamber C arranged at the center of 40 the distilling chamber A and having its lower end communicating with an eduction pipe D which is connected with a suction-producing device (not shown) and a plurality of devices E projecting radially from 45 the take-off duct into the body of material in the chamber A and so constructed that they form unobstructed passageways 1 that extend from the take-off duct C through the coking zone and into the material lying out- 50 side of the coking zone that has passed through the coking stage. The particular construction and arrangement of the devices E is immaterial, so long as they provide unobstructed passageways that extend through 55 the coking zone and establish communica- 60 tion between the take-off duct C and the portion of the distilling chamber lying outside of or beyond the coking zone without liability of causing the suction in the take-off duct being exerted on the outer side of the 65 barrier of solidifying material that surrounds the molten mass in the coking zone. I prefer, however, to form the devices E from short tubular members screwed into the take-off duct C or connected to same in 70 any other suitable manner and provided with openings 1<sup>a</sup> through which the gases and vapors can enter the passageways 1. In the apparatus herein shown the members E are closed at their outer ends and are 75 provided on their undersides with slots 1<sup>a</sup> that extend longitudinally of said members, and thus permit the gases to enter the passageways 1 at any point throughout the 80 length of said passageways.

When heat is applied to the walls of the distilling chamber A the material in said chamber will become coked progressively, as the heat penetrates inwardly through said material. As the coal begins to heat it 85 softens and starts to give off gases and oils. The oils are light in gravity and very volatile, and the gases are high in methane, most of the moisture in the coal being driven off at this period in the carbonization. The 90 coal begins to melt as the temperature is elevated, and after it has been partially melted, it is of putty-like consistency and almost 95 impervious to the passage of gases and vapors, due to the fact that little of it has 100 been decomposed into the more solid products formed later in the distilling operation. The pitchy oils which result from the 105 partial decomposition of the coal completely fill the voids between the pieces of coal, and being very viscid, offer great resistance to the passage of the volatile products which 110 have resulted from the decomposition of the coal lying closer to the source of heat that has undergone more nearly complete 115 decomposition. The melted, pitch saturated coal gives off considerable gases, but due to the fact that condensation of the heavier fractions from the more completely carbonized zone occur, the evolution is somewhat retarded and only the hydrocarbons of a lighter gravity and the permanent gases escape from the decomposing coal in this 120 zone. Located immediately adjacent to this zone, but toward the side wall of the retort 125 to which the heat is applied, the coal is a boiling, bubbling mass. The temperature of this mass is approximately 650° F. to 750° F., these temperatures indicating the beginning and ending of the reaction. It 130 is from this boiling, bubbling mass that most of the volatile matter escapes, and it is at this point that almost all of the oily hydrocarbons are formed and probably 50% of the gases evolved. Immediately outside

of the boiling, bubbling mass of melted coal is a thin, vertical layer of impervious, solidifying coke which separates the boiling, bubbling mass from the permanent coke or material that has passed through the coking stage. This thin vertical layer of solidifying coke is very dense and for a few moments after it has started to solidify it continues to give off its volatile matter, therefore gradually setting harder and harder into permanent coke. As previously stated, it is essential that this thin layer of solidifying material, constituting a barrier between the molten mass in the coking zone and the permanent coke lying outside of the coking zone, be kept intact, for any disturbance of same at the period when it is setting or becoming hard is bound to make the resultant coke fragile, filled with large bubbles, and in the form of small pieces. In Fig. 2 of the drawings I have used the reference character X to designate the boiling, bubbling mass in the coking zone that is passing through the coking stage, the reference character Y to designate the thin vertical barrier of solidifying coke that surrounds the molten mass in the coking zone and separates it from the material Z lying outside of the coking zone which has passed through the coking stage, and the reference character W to designate the material lying between the center take-off duct and the boiling, bubbling mass in the coking zone. In view of the fact that the vertical barrier Y is very thin, usually less than one-eighth of an inch in thickness, it has been herein represented by a solid line.

The devices E previously referred to that project radially from the center take-off duct, pass through the barrier Y that separates the molten mass X in the coking zone from the material Z that has passed through the coking stage. Consequently, any gases that continue to evolve from the material Z lying outside of the coking zone will travel inwardly through the passageways 1 in the devices E into the take-off duct C, thereby eliminating the possibility of the barrier Y being disrupted at the critical stage in the coking operation by the passage inwardly through same of gases that continue to evolve from the material that has passed through the coking stage, and also eliminating the possibility of pressure building up in the retort outside of the coking zone sufficiently to crack the retort.

The take-off duct can either be provided with numerous orifices 2 through which the gases, vapors and liquids evolved from the material in the coking zone and from the material lying within the coking zone are admitted to said take-off duct, or the radially-projecting devices E on the take-off duct can constitute the sole inlet into the

take-off duct for the evolved gases, vapors and liquids.

During the distilling operation the gases, vapors and liquids that evolve from the material passing through the coking stage are drawn inwardly into the take-off duct C by the suction or vacuum therein, said gases, vapors and liquids entering the take-off duct either through the perforations 2 therein or through the passageways 1 in the radially-projecting devices E. The gases, vapors and liquids that enter the take-off duct C travel downwardly through same to the eduction pipe D through which they are immediately conveyed away from the apparatus. In view of the fact that the take-off duct C is arranged at the center of the distilling chamber at the coolest part of the body of material in said chamber, the gases, vapors, and liquids that are evolved from the material which is passing through the coking stage will travel through the coolest portion of the material in the chamber. In escaping from said chamber, thus causing a reduction in the temperature of the gases, vapors and liquids below the initial temperature of formation, and consequently, preventing any further breaking down of the hydrocarbon molecules. As the liquids are immediately conducted out of the apparatus through a take-off duct which is so formed that no liquids can collect and remain therein, there is no possibility of the liquids condensing, revaporizing or becoming cracked or mixed with the material in the distilling chamber that surrounds the take-off duct C.

The gases, that continue to evolve from the material outside of the coking zone, also pass into the take-off duct through the passageways 1 extending through the coking zone. Consequently, there is no possibility of pressure building up in the retort outside of the coking zone X sufficiently to crack the retort or disrupt the thin barrier Y of solidifying material that separates the molten mass in the coking zone from the permanent coke. A relatively slight suction is employed to withdraw the gases, vapors and liquids from the retort,—in fact, only a suction of sufficient intensity to assist in collapsing the bubbles in the boiling mass in the coking zone and to overcome the resistance offered by the putty-like mass of partially melted coal and the mass of pitch saturated coal lying between the take-off duct and the coking zone. The suction should be great enough, however, to cause the escape into the passageways 1 of the gases that continue to evolve from the material lying outside of the coking zone that has passed through the coking stage, but not strong enough to cause the gases evolving in the coking zone to force their way

outwardly through the barrier Y. This desirable result is accomplished in my improved process and apparatus by reason of the fact that the gases which continue to evolve from the material lying outside of the coking zone are conducted into the center take-off duct through devices E which are of such a character that the fused material in the coking zone will seal itself around said devices during the coking operation, and which are so constructed that the permanent coke in the zone Z tends to obstruct the inlet slots 1<sup>a</sup> on the underside of the devices E, thereby creating a differential pressure on opposite sides of the barrier Y. In other words, in my process the gases that tend to disrupt the solidifying material in the coking zone are conducted out of the retort through unobstructed passageways penetrating through the coking zone, but entirely surrounded by fused coal which seals and cuts off any communication between the green coal and the permanent coke except through said passageways, thus preventing the suction or vacuum employed to withdraw the gases from acting on both sides of the barrier Y of solidifying material in the coking zone.

From the foregoing it will be seen that the process above described insures the production of a good grade of coke that is firm and in the form of large pieces; it eliminates the possibility of pressure building up in the retort outside of the coking zone sufficiently to crack the retort, if it be made of clay or silica, and it insures the recovery of a large percentage of the volatile constituents in the carbonaceous material being treated by the process.

In the apparatus herein shown the take-off duct C is provided at its lower end with a laterally-projecting flange 3 which supports or sustains the material in the distilling chamber A, and said take-off duct is arranged in the distilling chamber in such a manner that it is adapted to be drawn upwardly through said chamber to discharge the contents of the distilling chamber, the upper end of the distilling chamber being closed by a removable cover 4. In such an apparatus, namely, one in which the take-off duct sustains the charge, the radially-projecting devices E on the take-off duct have a dual function, namely, they permit the escape into the take-off duct of any gases that evolve from the material lying outside of the coking zone and they tend to hold the coked residue of the distilling operation on the take-off duct while said take-off duct is being withdrawn from the retort and conveyed away to the point where the coke is to be quenched or stored.

Having thus described my invention, what I claim as new and desire to secure by Letters Patent is:

1. A process for distilling, carbonizing or vaporizing solid carbonaceous material, characterized by subjecting a continuous body of material of the character mentioned to heat in a closed chamber, and withdrawing the evolved gases, vapors and liquids and maintaining the material in the coking zone in uninterrupted condition. 70

2. A process for distilling, carbonizing or vaporizing solid carbonaceous material, characterized by subjecting a continuous body of material of the character mentioned to heat in a closed chamber in such a manner that the material in said chamber becomes coked progressively, withdrawing the evolved gases, vapors and liquids by reduced pressure through the coolest portion of the material and conducting said gases, vapors and liquids out of the apparatus before secondary decomposition can occur and causing the gases that continue to evolve from the material that has passed through the coking stage to pass through the layer of solidifying material in the coking zone and escape from said chamber while maintaining the material in the coking zone in uninterrupted condition. 80 85 90

3. A process for distilling, carbonizing or vaporizing solid carbonaceous material, characterized by subjecting material of the character mentioned to heat in a closed chamber so as to liberate and drive off the volatile constituents, withdrawing the evolved gases, vapors and liquids, and providing unobstructed passageways in the barrier of solidifying material in the coking zone so as to permit the escape of any gases which continue to evolve from the material that has passed through the coking stage. 95 100

4. A process for distilling, carbonizing or vaporizing solid carbonaceous material, characterized by applying heat externally to a closed chamber containing a continuous body of material of the character mentioned, subjecting the material in the coking zone to the action of a suction of sufficient intensity to assist in the collapse of the bubbles in the molten mass in said zone and also withdraw the evolved gases, vapors and liquids, and causing the gases that continue to evolve from the material that has passed through the coking stage to escape from said chamber while maintaining the material in the coking zone in uninterrupted condition. 110 115 120

5. A process for distilling, carbonizing or vaporizing solid carbonaceous material, characterized by subjecting material of the character mentioned to heat in a retort or distilling chamber provided with a center take-off duct or collection chamber, providing and maintaining unobstructed passageways in said material that branch radially from said take-off duct, and creating a suction in said take-off duct of sufficient intensity to withdraw the evolved gases, vapors 125 130

and liquids without liability of disrupting the barrier of solidifying material that separates the molten mass in the coking zone from the material which has passed through the 5 coking stage.

6. A process for distilling, carbonizing or vaporizing solid carbonaceous material, characterized by applying heat externally to a chamber containing solid carbonaceous material, causing the gases, vapors and liquids that are evolved from the material passing through the coking stage to travel through the coolest portion of the material in said chamber into an off-take passageway and 10 providing unobstructed passageways in the body of material in said chamber, that branch radially from said off-take passageway at a plurality of levels and through which gases can travel into said off-take 15 passageway from the zone lying outside of the coking zone.

7. A process for distilling, carbonizing or vaporizing solid carbonaceous material, characterized by applying heat externally to a chamber containing solid carbonaceous material, causing the gases, vapors and liquids evolved from the material passing through the coking stage to travel through the coolest portion of the material in said chamber 20 into an off-take passageway and thence downwardly through said off-take-passageway, and providing unobstructed passageways in the body of material in said chamber that lead from said off-take passageway 25 outwardly through the coking zone so as to permit the escape of gases that continue to evolve from the material lying outside of the coking zone.

8. A process for distilling, carbonizing or 30 vaporizing solid carbonaceous material, characterized by applying heat externally to a chamber containing a continuous body of solid carbonaceous material, withdrawing under reduced pressure the gases, vapors 35 and liquids evolved from said material and causing said gases, vapors and liquids to travel through the coolest portion of the material in said chamber and thence immedi-

ately escape from the apparatus and providing unobstructed passageways, consisting 50 of independent ducts, at numerous points throughout the material in said chamber for the escape of gases that continue to evolve from the material which has passed through the coking stage.

9. A process for distilling, carbonizing or vaporizing solid carbonaceous material, characterized by externally heating a chamber containing a continuous body of solid carbonaceous material, causing the gases, vapors and liquids evolved from the material passing through the coking stage to travel through the coolest portion of the material in said chamber into a center take-off duct and thence flow downwardly through said 60 take-off duct to an eduction pipe and providing unobstructed passageways at numerous points throughout the body of material in said chamber in the form of independent ducts that branch laterally from 65 said take-off duct through the continuous barrier in the coking zone and which prevent pressure from building up in the chamber outside of the coking zone.

10. A process for distilling, carbonizing or vaporizing carbonaceous material, characterized by applying heat externally to a chamber containing solid carbonaceous material, causing the gases, vapors and liquids evolved from the material passing through the coking stage to travel into a center take-off duct through the coolest portion of the material in said chamber and through hollow members arranged at numerous points 80 throughout the body of material in said chamber which form unobstructed passageways that extend through the coking zone and establish communication between the take-off duct and the portion of said chamber lying beyond or outside of the coking zone, and causing the gases, vapors and liquids that enter the take-off duct to flow 85 downwardly through same to an eduction pipe.

GEORGE W. WALLACE